

Oct. 15, 1929.

J. J. NAUGLE

1,731,474

PROCESS FOR THE TREATMENT OF COMMINUTED CARBONACEOUS MATERIAL  
AND THE LIKE, IN ELECTRIC FURNACES AND THE LIKE

Filed April 21, 1923 2 Sheets-Sheet 1

Fig. 1.



Fig. 2.



Fig. 3.



INVENTOR

JOHN J. NAUGLE

Edward M. Erhart  
BY  
ATTORNEY

Oct. 15, 1929.

15, 1929. J. J. NAUGLE 1,731,474  
PROCESS FOR THE TREATMENT OF COMMINUTED CARBONACEOUS MATERIAL  
AND THE LIKE, IN ELECTRIC FURNACES AND THE LIKE  
Filed April 21, 1923 2 Sheets-Sheet 2

Filed April 21, 1923 2 Sheets-Sheet 2

Fig. 4.



Fig. 5.



Fig. 6.



Fig. 7.



**INVENTOR**

JOHN J. NAUGLE,

John C. WAGGONER,  
*Edward M. Erast*  
BY  
ATTORNEY

**ATTORNEY**

## UNITED STATES PATENT OFFICE

JOHN J. NAUGLE, OF BROOKLYN, NEW YORK

PROCESS FOR THE TREATMENT OF COMMINUTED CARBONACEOUS MATERIAL AND THE  
LIKE IN ELECTRIC FURNACES AND THE LIKE

Application filed April 21, 1923. Serial No. 633,643.

My present invention relates to methods of treating comminuted material, particularly comminuted carbonaceous material, such as comminuted carbonized lignin residues obtained by carbonizing the cooking liquors derived from the treatment of wood by the alkali (soda) process in the production of wood pulp, or such as spent decolorizing carbon, for the production from the materials designated of a pure grade of carbon characterized by a very low "ash" or mineral content, high electrical conductivity, and a remarkably high degree of activation corresponding to a high degree of decolorizing power. It is an object of the present invention to devise methods of the character specified above which shall be exceedingly simple in operation, requiring comparatively simple apparatus and a minimum of time, labor and material for this purpose, which shall produce the desired product in the desired condition of high purity, high conductivity and a high degree of activation and decolorizing power, which shall effect such a distribution of heat through the mass of material being treated, during the various stages of its treatment, as shall be best calculated to bring about the desired result in the most expeditious and reliable manner; and which shall render possible a very high yield of the desired end product by a continuous, rather than by a batch, process.

In the accompanying specification I shall describe an illustrative embodiment of the method of the present invention. In the accompanying specification I shall also describe, and in the annexed drawing show, one form of apparatus in which the method of the present invention may be conveniently practiced. It is, however, to be clearly understood that my invention is not limited to the specific embodiment of the process described herein, nor to the use of the particular form of apparatus shown and described herein, said apparatus forming the subject matter of a separate application for Letters Patent filed by me of even date herewith.

In order that my invention may be more clearly understood, reference may be made to a co-pending application of mine filed of

even date herewith, Serial No. 633,640 and entitled "Method of treating carbonaceous material in an electric furnace or the like."

In practicing the aforesaid illustrative embodiment of the method of the present invention, I first take any suitable raw material, preferably a carbonaceous material, in comminuted or finely divided form. While various types of comminuted carbonaceous material may be treated with success in accordance with the principles of the present invention, either in the production of a highly activated carbon from the raw material, or in the revivification of spent decolorizing carbon, I shall describe the present invention as applied more particularly to the purification of a highly activated carbon from carbonized lignin residues in comminuted form, such residues being obtained by carbonizing the cooking liquors derived from the treatment of wood by the alkali (soda) process in the production of wood pulp.

Taking, for example, the raw material specified above, which material comprises comminuted carbonized lignin residues, such material may have an average analysis as follows:

*Analysis of comminuted carbonized lignin residues*

|        | Per cent |
|--------|----------|
| Carbon | 90       |
| Ash    | 10       |

*Analysis of ash*

|                       |       |
|-----------------------|-------|
| Silicious matter      | 0.13  |
| Silica                | 0.75  |
| Ferric oxide          | 0.34  |
| Alumina               | 0.47  |
| Lime, CaO             | 0.23  |
| Magnesia, MgO         | 0.11  |
| Chlorine as chlorides | 0.47  |
| Sulphuric anhydride   | 2.65  |
| Carbon dioxide        | 1.00  |
| Alkalies (by diff.)   | 3.85  |
|                       | 95    |
|                       | 10.00 |

This material contains certain volatile matter and also certain fusible mineral substances which have a high electrical resistance and

which serve substantially to reduce the conductivity of the raw material.

I now heat the mass of raw material specified above so as to expel the volatile substances and to fuse the contained mineral substances, characterized by a high resistivity, for the subsequent removal of such fused mineral substances. This I preferably do by subjecting the raw material to the successive action of degrees of heat of varying intensities. While the process may be carried out by successively subjecting the raw material to degrees of heat which are relatively increasing, I have found that to subject the material to successively decreasing stages of heat is eminently as satisfactory but I do not wish to be confined to this particular method. In accordance with this statement I will describe the process in which the degrees of heat to which the material is successively subjected diminish during each successive stage of treatment. For example, if the material is subjected to three successive stages of heat treatment, it may be heated to a temperature from 800° to 1500° C. in the first stage, from 600° to 1200° C. in the second stage, and from 400° to 600° C. in the third and last stage, where a highly activated decolorizing carbon is manufactured from the raw material specified; or up to 600° C. in the first stage, up to 500° C. in the second stage, and up to 400° C. in the third and last stage, where spent decolorizing carbons are treated for revivification.

In order to effect the desired heat treatment of the raw material in the successive stages, corresponding to successively diminishing degrees of heat, I prefer to subject such material to the successive action of electric currents of varying, such as diminishing, densities. Such electric currents should preferably be passed directly through the raw material during its treatment. For example, in the first stage of treatment for the manufacture of a highly activated decolorizing carbon, a comparatively high current density should be employed, while in the second stage of the treatment a moderate current density should be employed; and in the third and last stage of the treatment a comparatively low current density should be used.

In carrying out the process, the material is continuously fed into the successive heating chambers so as to be subjected to the electric currents of varying, such as diminishing, densities for generating degrees of heat of correspondingly varying, such as diminishing, intensities. Preferably, the current is passed into the material between relatively movable electrodes which serve to effect an intimate mixture and stirring action of the material being treated. Feeding means may be provided within the heating chambers to continuously advance the material during the successive stages of treatment and to feed the material from one heating chamber to the

next, thus subjecting the material being treated to successive sets of electrodes for passing electric currents through the material in contact with the particular set of electrodes.

The heat treatments described effect a substantial elimination of volatile substances present in the raw material being treated and serve also to fuse the fusible mineral substances present in the mass being treated, which mineral substances, when fused, are found to adhere to the electrodes or to other parts of the apparatus, and are thus removed from the material being treated in accordance with the principles of the present invention. The removal of such mineral substances, characterized by a high electrical resistivity, serves to substantially increase the conductivity and purity of the treated product, and thus to yield a product having a correspondingly high degree of activation and decolorizing power.

The present method may be combined with considerable success with the means and method described and claimed in my copending application, filed May 22, 1922, Serial No. 562,828, and entitled "Prefiltering means and method," especially so far as the preliminary treatment of the raw materials is concerned, particularly to effect, as by decantation from a watery suspension of such material, a more or less partial preliminary separation by gravity of the portions of the material richer in carbon from the portions of the material poorer in carbon and containing an excess of heavy mineral substances. I may also use the feature of effecting a purification of the final product by forced filtration, under pressure, through a layer of the final product, of an aqueous acidified fluid and of wash waters. I may also add to the charge of material being treated in accordance with the principles of the method of the present invention certain reagents, such as sodium fluoride, which will have the property of eliminating one or more of the mineral substances present in the charge, particularly silica, in the form of volatile by-products, such as silicon fluoride.

In the practice of the foregoing method, I may also provide means for eliminating the gaseous products of the reaction continuously, or from time to time, and I may also provide means for testing the product during each of the stages of its treatment in accordance with the method of the present invention. I may also provide means for introducing an atmosphere of any desired gas into the apparatus in which the process is being carried out. If desired, this gas may be either a neutral gas, such as nitrogen, calculated to diminish combustion of the material treated, if such material is combustible, or may be some gas intended to react with some of the impurities present in the material being treated so as to yield a final product of the

maximum purity, electrical conductivity and activation and decolorizing power.

The resulting product possesses many advantages for the intended purpose, since it can be very cheaply made in accordance with the method of the present invention, and possesses the desired quality of high conductivity, corresponding to a remarkably high degree of activation and decolorizing power.

10 An average analysis of such material is as follows:

*Analysis of the final product*

|                                                                     | Per cent   |
|---------------------------------------------------------------------|------------|
| Carbon                                                              | 97.60      |
| 15 Ash                                                              | 2.40       |
| <i>Analysis of ash</i>                                              |            |
| Calcium                                                             | 0.16       |
| Sodium, $\text{Na}_2\text{O}$                                       | 0.35       |
| 20 Magnesium, $\text{MgO}$                                          | 0.16       |
| Chlorides, $(\text{Cl}_2)$                                          | 0.06       |
| Sulphates ( $\text{SO}_4$ )                                         | 0.78       |
| Silica, $\text{SiO}_2$                                              | 0.50       |
| Iron and alumina ( $\text{Fe}_2\text{O}_3, \text{Al}_2\text{O}_3$ ) | 0.39       |
| 25                                                                  | <hr/> 2.40 |

This product is also characterized by a very high degree of purity, corresponding to a high electrical conductivity and a high degree of activation and decolorizing power. The conductivity of the final product is often increased as much as five times that of the raw material treated, and its mineral content is often reduced to as low as one-fourth or less than that of the raw material treated in accordance with the method of the present invention. The method itself is exceedingly simple to practice, requiring comparatively simple apparatus and a minimum of time, labor, power and material for this purpose. The method is also admirably calculated to produce the desired end product in the desired condition of purity, high conductivity and high degree of activation and decolorizing power. This method is also very economical in view of the very high yield which may be obtained by its practice as compared with the methods hitherto employed for revivifying spent decolorizing carbon or for producing highly activated carbons for decolorizing purposes from the raw materials.

Referring to the drawing, wherein I have illustrated one form of apparatus in which the method outlined above may be conveniently practiced:

Fig. 1 is a side view, partly broken away, showing the aforesaid furnace in which the aforesaid illustrative embodiment of the method of the present invention may be practiced with considerable success;

Fig. 2 is a longitudinal sectional view of the same, partly in elevation;

Fig. 3 is a cross sectional view, partly in elevation, taken along line 3-3 of Fig. 2 of the drawing;

Fig. 4 is a side view of one form of central or inner electrode which may be used with the aforesaid furnace;

Figs. 5 and 6 are enlarged detail views of the electrode shown in Fig. 3 of the drawings; 70

Fig. 7 is a side view, partly diagrammatic, indicating one form of wiring circuit that may be used in connection with the aforesaid furnace. 75

Referring now to the aforesaid form of furnace, and more particularly to the drawing illustrating the same, said furnace includes a casing, generally indicated by reference character 10 and being preferably of substantially cylindrical form. The casing 10 comprises a plurality of, here shown as three, sections 11, 12 and 13, these sections being made of metallic material, such as cast iron or steel, and serving as the external electrodes of the device, as subsequently described in greater detail. 80

At 14 I have shown an inlet provided with a suitable type of feeding means, such as the feed hopper generally indicated by reference character 15 and including the feeding member 16 rotatably operated from any suitable source of power, not here deemed necessary to be shown. At the outlet end of the machine, I have provided a discharge hopper 95 17 communicating with a discharge chute 18 leading to any suitable bin or other storage device in which the finished material may be stored.

Each of the sections 11, 12 and 13 is provided with the flanged ends 19, 19; 20, 20; and 21, 21, respectively, while the inner ends of the inlet 14 and the outlet 17 are provided with the flanged ends 22 and 23, respectively. Insulating gaskets 24 are inserted between the meeting faces of the flanged ends just referred to, so that the successive sections 11, 12 and 13 of the casing 10 will be insulated from each other and from the inlet 14 and the outlet 17. 100

Suitably mounted for rotation within the casing 10 is an inner electrode or shaft generally indicated by reference character 30. The shaft 30 is also divided into a series of, here shown as three, sections 31, 32 and 33, 115 corresponding in number to the sections 11, 12 and 13 of the casing 10. Each of the sections 31, 32 and 33 is provided with a series of conducting vanes or electrodes 34 which are preferably integral with the respective 120 sections of the shaft 30.

One end 35 of the shaft 30 passes through the collar 36 forming an extension of the inlet 14 and preferably integral therewith. The other end 37 of the shaft 30 passes 125 through a similar collar 38 forming an extension of the outlet 17 and being preferably integral herewith. Preferably, the ends 35 and 37 of the shaft 30 are insulated from the collars or extensions 36 and 38, respectively, 130

so that the shaft 30, and the sections 31, 32 and 33 of which the same is composed, including also the conducting vanes or electrodes 34, are insulated from the casing 10, including the sections 11, 12 and 13, of which the same is composed, and including, also, the inlet 14 and the outlet 17.

The section 31 has a plurality of flanged portions 39 and 40 at its ends, while the section 32 is provided with the flanged end portions 41, 41, the section 33 being provided with the flanged portions 42 and 43 at its ends. Gaskets 44 are inserted between the opposed flanged end portions of the sections 31, 32 and 33 of the shaft 30, so that the various sections of the shaft will be insulated from each other. The section 31 is preferably hollow so as to permit the passage therethrough of an auxiliary cable or conductor 45 which is insulated from the section 31 and also from the section 33, but which is in electrical connection at its inner end, as indicated at 46, with the intermediate section 32, and at its outer end, as indicated at 47, with a flanged sleeve or thimble 48 carried by the shaft 45, but insulated therefrom, all for a purpose subsequently to be described in greater detail.

Within the casing 10 are means generally indicated by reference character 50 for efficiently mixing and stirring the material treated in the furnace, and for continuously advancing the same from one heating zone to the next during the treatment. While various devices may be employed for this purpose, I prefer to employ the means shown in the drawing, preferably Fig. 2 of the same, and comprising a plurality of spiral elements 51 carried by the successive sections 31, 32 and 33 of the shaft 30, as by means of the supporting arms of brackets 52. As shown in Fig. 3 of the drawing, the arms or brackets 52 are supported at their inner ends 53 by the respective sections 31, 32 and 33 of the shaft 30, and carry at their outer ends, indicated by reference character 54, the spiral elements 51 of the feeding means 50. It will also be noted that in the form illustrated, three spiral elements 51 are required for one complete turn of the spiral feeding means 50. Preferably, the spiral feeding means 50 and the arms or brackets 52 supporting the same, are of insulating material, or covered with insulating material, so as not to serve as current carriers.

At 60 I have shown an exhaust pipe, communicating by means of the connection pipes 61, 62 and 63, with the successive sections 11, 12 and 13 of the casing 10. The exhaust pipe 60 leads to a condenser and a water seal, so as to serve as an exhaust for the gaseous products of combustion or reaction, or for any other gas which may be present or which may be admitted to the charge within the furnace.

At 70 I have indicated a tube communicating, by means of the connections 71, 72 and

73, with the successive sections 11, 12 and 13 of the casing 10. The gas inlet tube 70 may be connected with a source of supply of gas, preferably under pressure, intended to be directed to the charge within the furnace. 70 This gas may be either a neutral gas, to provide an inactive atmosphere within the furnace to lessen combustion, such as nitrogen gas, for example, or may be some other gas intended to take part in the reaction within the furnace, as to serve to eliminate in gaseous form certain undesirable impurities present in the charge of material within the furnace. 75

At 81, 82 and 83 I have indicated sample test holes provided with the covers 84, 85 and 86, respectively, permitting the charge within each of the furnace sections 11, 12 and 13 to be sampled and examined from time to time, so as to determine the condition of the charge within the furnace at its different stages of treatment. 80

In order to provide proper electrical connections for the electrodes comprising the case sections 11, 12 and 13, and the sections 31, 32 and 33 of the shaft 30 carrying the conducting vanes or electrodes 34, I may employ the means shown more clearly in Figs. 4 and 7 of the drawing, and comprising the brushes 91, 92 and 93 contacting with the annular ends 39, 43 and 48 of the shaft sections 31 and 33, and the conducting thimble 47, respectively. The brushes 91, 92 and 93 are connected, by means of the wires 94, 95 and 96, with one of the poles, such as the positive pole, of a direct current generator of suitable capacity, this generator being preferably provided with a shunt wound field. The casing sections 11, 12 and 13 are connected, at the points 11', 12' and 13', with the wires 97, 98 and 99, leading to the remaining pole, that is, the negative pole, of the shunt wound generator referred to, which generator is not here deemed necessary to be shown. This system of electrical distribution is more particularly described and claimed in an application which will be filed. 95 100 105 110

In order to effect a relative movement, such as a relative rotation, of the cooperating sets of electrodes each comprising a casing section and a shaft section carrying the conducting vanes or electrodes 34, I employ any suitable means for effecting the desired relative movement, such as the spiral gear 100 cooperating with the worm 101 driven from any suitable source of power, not here deemed necessary 120 to be shown. By the operative engagement of the worm 101 with the spiral gear 100, the shaft 30, comprising the sections 31, 32 and 33, carrying the conducting vanes or electrodes 34, is rotated at any suitable rate of speed relatively to the casing 10 comprising the casing section 11, 12 and 13. The feeding means 50, in the form of the plurality of spiral feeding elements described above, being carried by the shaft 30, will likewise 125 130

be rotated with the same, and will thus serve to feed or advance the material during the treatment and also to assist in thoroughly stirring and mixing the same.

5 The manner of assembling the above machine will be substantially clear from the foregoing description. The manner of operating the machine will also be substantially clear from the foregoing description and may 10 be briefly summarized as follows: In commencing the operation of the furnace, the material to be treated, such as the comminuted carbonized lignin residues referred to, is fed into the feed hopper 15 and is thereupon continuously fed into the inlet 14 of the machine 15 by means of the rotating feeding element 16. From the inlet 14 the material to be treated is fed into the first of the heating zones or reaction chambers, in this case the 20 heating zone or reaction chamber within the casing section 11. From the section 11 the material is fed into the successive heating zones or chambers within the successive casing sections 12 and 13, by means of the feeding 25 means 50.

By the operation of the gears 100 and 101, the shaft 30, comprising the shaft section 31, 32 and 33 carrying the conducting vanes or electrodes 34, is caused to rotate with respect 30 to the sections 11, 12 and 13 of the casing. At the same time, the feeding means 50, also carried by the shaft 30 and the sections thereof, is caused to rotate, thus causing the rotation and operation of the spiral feeding elements 51, which, together with their supporting arms 52, are insulated from the shaft 30 and the sections 31, 32 and 33 of the same, and also from the conducting vanes or electrodes 34, as well as from the casing 10 and 35 the casing sections 11, 12 and 13 of the casing 10. This relative rotation causes the material being treated, here designated by reference character M, to be continuously fed from one heating zone or reaction chamber into the 40 next, and to be thus subjected to electric currents of varying densities and correspondingly varying degrees of heat. In the present instance, for the particular purpose in view, the current densities, and thus the degrees of 45 heat, diminish from one heating zone or reaction chamber to the next, in the direction of the feed of the material being treated.

The time of treatment may vary, but is 50 usually from about 15 to 60 minutes. The treatment should be continued long enough to expel substantially all of the volatile matters contained in the raw material, and to fuse the fusible mineral substances present therein to the condition of small aggregates or clinkers. These will be found to adhere to the sections 31, 32 and 33 of the shaft 30, and to the conducting vanes or electrodes 34 carried thereby, as well as to the spiral feeding elements 51, and occasionally to the inner walls 55 of the sections 11, 12 and 13 of the casing 10.

The products of combustion are drawn off through the gas outlet 60 by means of the connecting tubes 61, 62 and 63 communicating with the respective casing sections 11, 12 and 13. The products of combustion or other 70 gases or reaction are led to a condenser and a water seal. By means of the pipe 70 having the connecting tubes 71, 72 and 73 communicating with the respective sections 11, 12 and 13 of the casing 10, I may admit a suitable 75 gas to the various reaction chambers, such as nitrogen gas, if it is desired to minimize combustion and to carry on the reaction in a neutral or inactive atmosphere, or some other gas or gases which it may be desired to add 80 and which will take part in the reaction, such as a gas calculated to remove in gaseous form some of the impurities present in the raw material being treated.

By means of the sample test holes 81, 82 85 and 83, provided with the respective covers 84, 85 and 86, I may withdraw samples from each of the heating zones or reaction chambers from time to time to determine the condition 90 of the material being treated in each of its stages. In this way I am enabled to regulate the speed of feeding the material into the machine; the rate at which the material should be fed through the machine and be mixed and stirred; and also the current densities and 95 heat intensities which should best be employed with the particular material being treated in the machine. The finished product passes out of the machine through the outlet 17 into the discharge hopper 18, leading to a 100 bin or other suitable storage receptacle.

It may here be stated that the carbonized lignin residues referred to herein are the residues remaining after leaching the residues obtained by carbonizing the spent or used 105 cooking liquors derived in the treatment of wood by the alkali (soda) process in the production of wood pulp; and that the terms "activation" and "decolorizing", or their equivalents, as used in the specification and 110 claims, include also deodorization, purification and filtration.

It may also be stated that the heat treatment to which the raw material, such as the carbonized lignin residues referred to, is subjected, serves also to volatilize a part, at least, of the more readily volatile mineral constituents of the material being treated to produce the product of the present invention. The product is thus of an unusually high degree of 120 purity and of comparatively low specific gravity, weighing as low as about six, and up to about nine, pounds per cubic foot, whereas the raw material weighs from about eighteen down to about ten, pounds per cubic foot. 125 The product is also remarkably porous, of very uniform quality, and of very high efficiency.

Since I prefer, also, that the carbon of the present invention shall, in the course of its 130

preparation, or otherwise, be deprived of a substantial part of the "fines" or finer particles, the presence of which would tend to make the product unstable, to render it more combustible and to diminish its efficiency, which "fines" usually comprise from about twenty, to about thirty, per cent of the weight of the material treated for the production of the product which may be made with a high yield, which is remarkably stable, which is less combustible than other products of a similar nature, which shows a very low percentage of loss during its manufacture and during its use for filtration and subsequent 15 revivification, and which tends to yield a product of constantly increasing efficiency during successive revivifications.

This reduction in the percentage of "fines", or finer particles, may be effected by admitting air in regulated quantities through the inlet pipe 70 and the branches 71, 72 and 73 of the same leading to the casing sections 11, 12 and 13, respectively. The amount of air, or other oxidizing or oxygen-containing 25 gases, admitted to the heating or reaction chambers within the casing sections 11, 12 and 13 may be regulated by the respective valves 71', 72' and 73'. This amount of air, or its equivalent, may vary for the different chambers, since a greater degree of combustion will generally be desired in the first reaction chamber 11 than in the subsequent reaction chambers 12 and 13. It may here be stated that the heat of combustion resulting from the burning 35 of the "fines" referred to, assists in the treatment of the carbon and reduces the amount of electric current which would otherwise be required to generate the desired degree of heat in each of the reaction chambers. 40 The addition of air, or its equivalent, in regulated quantities, as above set forth, is found to have a very beneficial action upon the product, accelerating the reaction and acting, in some way, to produce a product of greater 45 purity, apparently by the elimination of some of the more volatile mineral constituents of the raw material being treated for the production of the final product.

Instead of air, or, sometimes, together with 50 air, or in place thereof, as by subjecting the material being treated to alternate treatments with air and steam, steam in regulated quantities may likewise be admitted to the respective reaction chambers within the casing sections 55 11, 12 and 13, through the inlet pipe 70 and the branches 71, 72 and 73 of the same controlled by the respective valves 71', 72' and 73'. Steam in some way acts to accelerate the reaction, as by breaking down the mineral substances present in the raw material being 60 treated, in this way yielding a product of increased porosity and purity. I may also add to the charge within the furnace an addition agent, such as a fluoride, as sodium fluoride, 65 for example, which would tend to combine

with a part or all of the mineral impurities present in the charge within the furnace, particularly silicious mineral impurities, such as silica and silicates, to produce volatile compounds which would thus be eliminated from the final product. Where the mineral impurity desired to be eliminated is silica, and the addition agent sodium fluoride, silicon fluoride is eliminated, with the production of a soluble byproduct which may be eliminated by washing the product. It may also be pointed out that the casing sections 11, 12 and 13 may be of different lengths, thus permitting the raw material to be subjected to treatment for different lengths of time in the respective reaction chambers, depending upon the particular treatment desired to be given such material in the particular chambers and under the particular atmospheric conditions, as to air, steam and products of combustion or other reaction, or otherwise, prevailing in the particular reaction chambers.

For the purpose of comparing the specific resistivity, or conductivity, as desired, of the raw material and of the final product, it may be stated that the total resistance of a mass of the raw material (in this case the carbonized lignin residues referred to) within a tube one inch long and one and seven-sixteenth inches in diameter, under a total pressure of one kilogram, was found to be about 167 ohms, corresponding to a resistance of about 6.28 ohms per cubic centimeter. The total resistance of a mass of the final product within a tube of the same dimensions and under a similar total pressure, was found to be about 33.5 ohms, corresponding to a resistance of about 1.26 ohms per cubic centimeter.

Another very valuable characteristic of the product of the present invention is that it is almost absolutely neutral, being neutral to phenolphthalein. This is probably the result of the manner in which the carbon is preferably produced, which consists in initially subjecting the raw material to a comparatively high temperature, which apparently converts the sulphates present in the raw material being treated, principally calcium and sodium sulphates, into sulphides, by the reducing action of the carbon, the sulphides, at a comparatively low temperature, being converted into the normal carbonates of calcium and sodium, respectively, to yield a neutral carbon. If the temperature is again raised so as to be comparatively high, the carbonates are apparently calcined and converted into the highly alkaline oxides. This is to be avoided since the neutralization of such an alkaline carbon by the addition of acid will tend to yield an acid carbon, which is highly undesirable, since acid carbons tend to invert sugar, where the carbons are used for the purification or filtration of sugar solutions, while alkaline carbons tend to form slimes which retard the rate of filtration or purifi-

cation; while the carbon of the present invention, being, as it is, absolutely neutral, no slimes tend to be formed and thus a high rate of filtration or purification is possible, while the absence of acid in the carbon avoids the inversion of sugar if sugar solutions are purified or filtered through the product of the present invention.

What I claim as my invention is:

1. The process of treating comminuted carbonaceous material, which comprises subjecting such material to the successive action of electric currents of relatively varying densities.

2. The process of treating comminuted carbonaceous material, which comprises subjecting such material to the successive action of electric currents of diminishing densities.

3. The process of treating comminuted material, which comprises passing through such material a succession of electric currents of relatively different densities.

4. The process of treating comminuted material, which comprises passing through such material a succession of electric currents of decreasing densities.

5. The process of treating comminuted material, which comprises stirring such material while passing through such material a succession of electric currents of decreasing densities.

6. The process of treating comminuted carbonaceous material, which comprises continuously advancing such material while subjecting such material to the successive action of electric currents of diminishing densities.

7. The process of treating comminuted material, which comprises continuously stirring and advancing such material while passing through such material a succession of electric currents of relatively different densities.

8. The process of treating comminuted carbonaceous material, which comprises advancing and stirring such material while subjecting such material to the successive action of electric currents of relatively varying densities.

9. The process of treating comminuted carbonaceous material containing fusible mineral substance, which comprises continuously advancing such material while subjecting such material to the successive action of electric currents of diminishing densities and removing fused mineral substance from such material.

10. The process of treating comminuted material containing fusible mineral substance, which comprises stirring such material while passing through such material a succession of electric currents of decreasing densities and continuously removing fused mineral substance from such material.

11. The process of treating comminuted material containing fusible mineral sub-

stance, which comprises passing through such material a succession of electric currents of relatively different densities and removing fused mineral substance from such material during each of the successive stages of subjection of such material to the action of the electric currents of different densities.

12. The process of treating comminuted carbonaceous material containing fusible mineral substance, which comprises advancing and stirring such material while subjecting such material to the successive action of electric currents of relatively varying densities and continuously removing fused mineral substance from such material during each of the successive stages of subjection of such material to the action of electric currents of varying densities.

13. The process of treating comminuted carbonaceous material containing fusible mineral substance, which comprises subjecting such material to the successive action of electric currents of relatively varying densities and removing mineral substance from such material.

14. The process of treating comminuted carbonaceous material containing fusible mineral substance, which comprises subjecting such material to the successive action of electric currents of diminishing densities and removing mineral substance from such material during each of the successive stages of subjection of such material to the action of the electric currents of diminishing densities.

15. The process of treating comminuted material containing fusible mineral substance, which comprises continuously stirring and advancing such material while passing through such material a succession of electric currents of relatively different densities and continuously removing mineral substance from such material during each of the successive stages of subjection of such material to the action of electric currents of different densities.

16. The process of treating comminuted material containing fusible mineral substance, which comprises passing through such material a succession of electric currents of relatively different densities and continuously removing mineral substance from such material.

17. The process of treating comminuted carbonaceous or like material containing fusible mineral substances, which comprises subjecting such material to the successive action of relatively varying degrees of heat and simultaneously removing fused mineral substance from such material.

18. The process of treating comminuted carbonaceous or like material containing fusible mineral substances, which comprises subjecting such material to the successive action of diminishing degrees of heat and continuously removing fused mineral substance

from such material during each of the successive stages of subjection of such material to the action of the diminishing degrees of heat.

19. The process of treating comminuted carbonaceous or like material containing fusible mineral substances, which comprises stirring such material while subjecting such material to the successive action of varying degrees of heat and removing fused mineral substance from such material during each of the successive stages of subjection of such material to the action of varying degrees of heat.

20. The process of treating comminuted carbonaceous or like material containing fusible mineral substances, which comprises continuously advancing and stirring such material while subjecting such material to the successive action of diminishing degrees of heat and continuously removing fused mineral substance from such material.

21. The process of treating comminuted carbonaceous and like material containing fusible mineral substances, which comprises passing such material from one heating zone to another heating zone of lesser heat intensity, and removing fused mineral substance from such material.

22. The process of treating comminuted carbonaceous and like material containing fusible mineral substances, which comprises continuously passing such material through a succession of heating zones of varying heat intensity, and continuously removing fused mineral substance from such material.

23. The process of treating comminuted carbonaceous and like material containing fusible mineral substances, which comprises passing such material from one heating zone to another heating zone of lesser heat intensity while stirring such material and removing fused mineral substance from such material in each of said heating zones.

24. The process of treating comminuted carbonaceous and like material containing fusible mineral substances, which comprises continuously passing such material through a succession of heating zones of varying heat intensity while continuously stirring such material and continuously removing fused mineral substance from such material in each of said heating zones.

25. The process of treating comminuted carbonaceous material containing substances of comparatively low electrical conductivity, which comprises continuously advancing such material while subjecting such material to the successive action of electric currents of diminishing densities and removing substances of comparatively low electrical conductivity from such material.

26. The process of treating comminuted material containing substances of comparatively high electrical resistance, which comprises passing through such material a suc-

cession of electric currents of relatively different densities and removing substances of comparatively high electrical resistance from such material during each of the successive stages of subjection of such material to the action of the electric currents of relatively different densities.

27. The process of treating comminuted carbonaceous material containing substances of comparatively high electrical resistance, which comprises subjecting such material to the successive action of electric currents of relatively varying densities and removing substances of comparatively high electrical resistance from such material.

28. The process of treating comminuted material containing substances of comparatively low electrical conductivity, which comprises continuously stirring and advancing such material while passing through such material a succession of electric currents of relatively different densities and continuously removing substances of comparatively low electrical conductivity from such material during each of the successive stages of subjection of such material to the action of electric currents of relatively different densities.

29. The process of treating comminuted carbonaceous or like material containing substances of comparatively high electrical resistance, which comprises subjecting such material to the successive action of varying degrees of heat and removing substances of comparatively high electrical resistance from such material.

30. The process of treating comminuted carbonaceous and like material containing substances of comparatively low conductivity, which comprises passing such material from one heating zone to another heating zone of lesser heat intensity, and removing substances of comparatively low conductivity from such material.

31. The process of treating comminuted carbonaceous material, which comprises subjecting such material to the successive action of electric currents of varying densities in the presence of an oxidizing gas.

32. The process of treating comminuted material, which comprises passing through such material a succession of electric currents of decreasing densities in the presence of air.

33. The process of treating comminuted carbonaceous material, which comprises continuously advancing such material while subjecting such material to the successive action of electric currents of diminishing densities in the presence of steam.

34. The process of treating comminuted carbonaceous material containing fusible mineral substance, which comprises continuously advancing such material while subjecting such material to the successive action of electric currents of diminishing densities in the presence of a regulated amount of an

oxidizing gas and removing fused mineral substance from such material.

35. The process of treating comminuted material containing fusible mineral substance, which comprises passing through such material a succession of electric currents of relatively different densities in the presence of a regulated amount of air and removing fused mineral substance from such material during each of the successive stages of subjection of such material to the action of the electric currents of relatively different densities.

36. The process of treating comminuted material containing fusible mineral substance, which comprises continuously stirring and advancing such material while passing through such material a succession of electric currents of relatively different densities in the presence of a regulated amount of steam and continuously removing mineral substance from such material during each of the successive stages of subjection of such material to the action of relatively electric currents of different densities.

37. The process of treating comminuted carbonaceous or like material containing fusible mineral substances which comprises subjecting such material to successive stages of relatively varying degrees of heat in the alternate presence of air and steam and removing fused mineral substance from such material, during each of said successive stages.

35. In testimony, whereof, I have signed my name to this specification this 30th day of March, 1923.

JOHN J. NAUGLE.

40

45

50

55

60

65